# EUROPEAN PATENT SPECIFICATION

(11) **EP 4 278 070 B1**
(45) Date of publication and mention of the grant of the patent: **25.02.2026**
(21) Application number: 22700539.4
(22) Date of filing: 10.01.2022
(51) Int. Cl.: F01D 5/20, F01D 11/12

(54) **PRE-SINTERED PREFORM WITH HIGH TEMPERATURE CAPABILITY, IN PARTICULAR AS ABRASIVE COATING FOR GAS TURBINE BLADES**
VORGESINTERTE VORFORM MIT HOCHTEMPERATURFÄHIGKEIT, INSBESONDERE ALS SCHLEIFBESCHICHTUNG FÜR GASTURBINENSCHAUFELN
PRÉFORME PRÉFRITTÉE À HAUTE TEMPÉRATURE, EN PARTICULIER COMME REVÊTEMENT ABRASIF POUR AUBE DE TURBINE À GAZ

(30) Priority: 14.01.2021 IT 202100000626
(43) Date of publication of application: 22.11.2023
(73) Proprietor: Nuovo Pignone Tecnologie - S.r.l., 50127 Florence (IT)
(72) Inventor: STRAMARE, Stefania, 50127 Florence (IT); TOGNARELLI, Leonardo, 50127 Florence (IT); MICHELASSI, Vittorio, 50127 Florence (IT); BALDI, Gino, 50127 Florence (IT); MASI, Gabriele, 50127 Florence (IT)
(74) Representative: Novagraaf Group
(86) International application number: PCT/EP2022/025007
(87) International publication number: WO 2022/152579

(56) References cited:
- EP-B1- 2 963 144
- GB-A- 2 551 527
- US-A1- 2015 118 060
- US-A1- 2016 069 195
- US-A1- 2018 311 772
- US-B2- 9 511 436

## Description

### TECHNICAL FIELD

The present disclosure generally relates to the field of turbomachines comprising high temperature components and to high resistance materials applied to such components, for example abrasive coatings and method of applying the same.

According to one embodiment, the present disclosure relates to axial, radial and mixed turbomachines, e.g. compressors and turbines, and more specifically to leakage control between the stationary and rotating components, and include abrasive materials applied to turbine rotor bucket or compressor rotor blade.

According to one embodiment, the present disclosure relates to abrasive coatings applied on rotor bucket tips to form a dynamic seal with the statoric part, called a shroud, to reduce the gas flow leakage and increase the efficiency of the gas turbine engine through the use of advanced materials and coatings with high temperature capability.

### BACKGROUND ART

GB 2 551 527 A discloses an abrasive coating for a gas turbine engine component. US 9 511 436 B2 discloses a composite composition for a turbine blade tip. US 2018/311772 A1 discloses a method of applying an abrasive. EP 2 963 144 B1 discloses an abrasive coating. US 2015/118060 A1 discloses a turbine engine blade. US 2016/069195 A1 discloses a rotary blade tip. US 2018/311772 A1 discloses a method of applying an abrasive. It is known that gas turbines generally include at least one stationary assembly extending over at least one rotor assembly. The rotor assembly includes at least one row of circumferentially spaced, rotatable, metallic turbine blades. The blades include metallic airfoils that extend radially outward from a rotatable hub to a metallic tip. Many of such metallic airfoils of rotor blades are fabricated from materials such as Nickel (Ni) based superalloys.

Stationary assemblies of turbomachines include surfaces that form metallic shrouds that may be routinely exposed to a hot gas flux. Some of such metallic surfaces include an applied metallic-based MCrAlY (where M = Co, Ni or Co/Ni, Cr = Chromium, Al = Aluminum and Y = Yttrium) coating and/or an applied ceramic thermal barrier coating that forms a shroud over the stationary assembly. Alternatively, some such metallic surfaces include applied ceramic matrix composites with, or without, a protective thermal barrier coating.

The metallic tips and the metallic shrouds define a tip clearance therebetween. However, such tip clearances are not suitable for high-temperature units that need high efficiencies. In order to reduce such tip clearances, gas turbines include abradable shrouds formed over the stationary assembly and the blade tips include an abrasive material formed thereon that has a greater hardness value than the blade material and the abradable coating. The abrasive material abrades the shroud coatings as the rotor assembly rotates within the stationary assembly. The abradable shroud coatings and the abrasive tips define a tip clearance therebetween. The tip clearance is small enough to facilitate reducing axial flow through the gas turbine that bypasses the blades, thereby facilitating increased efficiency and performance of the gas turbine. The tip clearance is also large enough to facilitate rub-free gas turbine operation through the range of available gas turbine operating conditions.

Various materials and processes have been suggested to provide a suitable abrasive tip cap on turbine stator and rotor blades. Typical abrasive materials used include silicon carbide, aluminum oxide, tantalum carbide and cubic boron nitride. The particles of abrasive material are usually incorporated with a metal matrix, including for example, nickel or cobalt-base alloys, to provide a sufficiently strong structure that can be bonded to the blade tip. However, the thickness of such a metal matrix is often limited because of the structural weakness of the abrasive composition.

In addition, some abrasive materials are damaged by high temperatures. As an example, for temperatures above approximately 927 °C (1700 °F), cubic boron nitride becomes unstable and is prone to oxidation. Also, while silicon carbide is better suited to survive temperatures in excess of approximately 927 °C (1700 °F), silicon carbide abrasives include free silicon that may attack the Ni/Co (Nickel/Cobalt) alloy substrates.

In some applications, it is conventional to apply the abrasive composition to the rotor blade tip using a thermal spray technique, such as plasma spraying or detonation gun spraying. Subsequent processes are typically necessary to provide the adhesion and structural integrity necessary for the abrasive composition to survive the hostile environment of a gas turbine. Such steps often include adhering the abrasive composition to the blade tip during a first heating and cooling cycle, and later depositing an additional quantity of the metal matrix over the abrasive composition through a second heating and cooling cycle, such as during hot isostatic pressing. As an alternative, it has also been suggested to melt the tip of the blade, such as with lasers, introduce the abrasive to the blade tip, and then re-solidify the blade tip.

While the above processes may be suitable for some turbine blade structures, turbine blade used in modern gas turbine engines are often fabricated from cast high temperature nickel-base superalloys having a single crystal microstructure. Single crystal blades are characterized by extremely high oxidation resistance and mechanical strength at elevated temperatures, which are necessary for the performance requirements of modern gas turbines. However, the single crystal microstructure must not be affected by the process by which the rotor blade abrasive tip caps are secured to the rotor blades. In particular, the process must not recrystallize the single crystal microstructure of the rotor blade, such that the high temperature properties of the rotor blade are lost or diminished. As a result, processes which entail melting the rotor blade tip to the single crystal rotor blade are entirely unacceptable. In addition, repeated thermal cycling of the rotor blade runs the risk of degrading the single crystal microstructure of the rotor blade.

Thus, it would be desirable to provide an abrasive composition which can be readily formed into an abrasive blade tip cap and which can be attached to a turbine rotor blade in a single heating and cooling cycle, under controlled temperature so as to minimize any degradation of the microstructure of a single crystal turbine rotor blade.

### SUMMARY

The present invention is defined in the accompanying claims. In one aspect, the subject matter disclosed herein is directed to an abrasive material preform configured to be fixedly coupled to a gas turbine rotor blade through a single heating and cooling cycle under controlled temperature.

In another aspect, the subject matter disclosed herein is directed to a method for producing such an abrasive material preform.

In yet another aspect, the subject matter disclosed herein is directed to a method for attaching such an abrasive material preform to a gas turbine blade in a single heating and cooling cycle to preserve the microstructure of a single crystal rotor blade and the stability of the abrasive material.

### BRIEF DESCRIPTION OF THE DRAWINGS

A more complete appreciation of the disclosed embodiments of the invention and many of the attended advantages thereof will be readily obtained as the same becomes better understood by reference to the following detailed description when considered in connection with the accompanying drawings, wherein:
Figure 1 illustrates a cross section of a gas turbine blade coated with an abrasive material preform;
Figure 2 illustrates a cross section of an abrasive material preform;
Figure 3 illustrates a flowchart of a new, improved method of making an abrasive gas turbine blade tip cap preform for bonding to a blade tip to form an abrasive blade tip cap on the tip of a gas turbine blade;
Figure 4 illustrates a flowchart of a new, improved method of applying an abrasive material preform on the tip of a gas turbine blade;
Figure 5 illustrates a flowchart of a first exemplary embodiment of the method of making an abrasive gas turbine blade tip cap preform of Figure 3;
Figure 6 illustrates a flowchart of a second exemplary embodiment of the method of making an abrasive gas turbine blade tip cap preform of Figure 3; and
Figure 7 illustrates a flowchart of an exemplary embodiment of the method of applying an abrasive material preform on the tip of a gas turbine blade of Figure 4.

### DETAILED DESCRIPTION OF EMBODIMENTS

In one aspect, the subject matter disclosed herein is directed to an abrasive material preform 11 configured to be fixedly coupled to a gas turbine rotor blade 10 through a single heating and cooling cycle under controlled temperature to realize a gas turbine blade 10 coated with an abrasive material preform 11 as shown in Figure 1.

According to one aspect, the subject matter disclosed herein is more specifically directed to a pre-sintered abrasive material preform 11 composed of a homogeneous mixture of a superalloy base material and braze alloy powders configured to be tack welded on a blade tip and then vacuum brazed, to realize a gas turbine blade 10 coated with an abrasive material preform 11 as shown in Figure 1.

In the present disclosure, the term powder is used according to its generally known meaning, to identify fine, dry, solid particles with mesh size between few to thousands of microns.

Additionally, in the present disclosure, the term sintering is also used according to its generally known meaning, to identify a process of compacting and forming a solid mass of material by heat or pressure without melting it to the point of liquefaction.

The term "preform" is used in the present disclosure to identify a preliminarily shaped component.

Figure 2 illustrates a section view of a pre-sintered preform 11, which is formed of two layers, namely a bonding layer 12, for coupling with a blade tip, and a top layer 13 or abrasive layer 13. According to an exemplary embodiment, thickness of each layer is 50%±15% of total preform thickness required for the application. In particular, according to an exemplary embodiment, the bonding layer 12 can be a metallic layer obtained by sintering a blend of a nickel braze alloy powder and a nickel base superalloy powder, as described in the following and the top layer 13 can be a ceramic layer in a metal matrix produced by sintering a blend of a cubic boron nitride (cBN) powder and an aluminum oxide (Al₂O₃) powder in a metal matrix of same composition of the bonding layer. The two layers may be obtained by a single sintering operation, or by a sequence of sintering operations, including the bonding of the separately sintered two layers.

According to an exemplary embodiment, a pre-sintered preform can be a sintered powder metallurgy product composed of a bonding layer 12 composed of a homogeneous mixture of superalloy base material and braze alloy powders and of a top layer 13 or abrasive layer 13 composed of abrasive powders, also called abrasive grits, with a composition within the ranges of Table 1.

**Table 1**

| ID | Powder Blend | Powder type | Weight (%) |
|---|---|---|---|
| 1 | Bonding | Ni based superalloy | 50 ± 15 |
| | | Ni based Braze alloy | 50 ± 15 |
| 2 | Abrasive | Cubic Boron Nitride (cBN) | 25 ± 7.5 |
| | | Aluminum Oxide (Al₂O₃) | 25 ± 7.5 |
| | | Bonding (see ID 1 ) | 50 ± 15 |

The metallic and abrasive powders are chosen to withstand high temperatures in gas turbine section. In particular, the abrasive grits ensure both short term cutting capability and thermal stability, assuring the clearance maintenance over time.

Powder particle size shall meet the following requirements:
- cBN powder particle size shall be in a range of 181-277 mesh in 93%wt minimum
- Al oxide powder particle size shall be 100 mesh in 40%wt minimum
- Ni based superalloy powder particle size shall be 395 mesh in 95%wt minimum
- Ni based braze alloy powder particle size shall be 395 mesh in 95%wt minimum

In an exemplary embodiment of the system, the composition of the nickel braze alloy powder is referred to in Table 2.

**Table 2**

| Element | Weight (%) |
|---|---|
| Nickel | 46,71 - 55,21 |
| Cobalt | 13.5 - 16.5 |
| Chromium | 18.5 - 21.5 |
| Aluminum | 4.2 - 5.8 |
| Silicon | 7.5 - 8.4 |
| Total other elements | < 1.1 |

In an exemplary embodiment of the system, the composition of the nickel based superalloy powder is referred to in Table 3.

**Table 3**

| Element | Weight (%) |
|---|---|
| Nickel | 55.61 - 60.36 |
| Cobalt | 11.35 - 12.1 |
| Chromium | 6.5 - 7.2 |
| Aluminum | 5.9 - 6.6 |
| Tantalum | 6.1 - 6.7 |
| Tungsten | 4.5 - 5.3 |
| Hafnium | 1.2 - 1.8 |
| Rhenium | 2.5 - 3.1 |
| Total other elements | < 1.6 |

According to an exemplary embodiment, a pre-sintered preform 11 is realized through the process shown in Figure 3, by forming 20 a tape or a sheet, which is formed of two layers, namely a bonding layer 12, and a top layer 13 or abrasive layer 13, with the composition specified above. The tape or sheet is then sintered, i.e. vacuum heat treated 30 to 80-90% of the brazing temperature and subsequently cut 40 to desired shape.

According to an exemplary embodiment, a pre-sintered preform 11 is coupled to a gas turbine blade tip through the process shown in Figure 4, by tack welding 50 the pre-sintered preform 11 to the tip of a gas turbine blade 10 and vacuum brazing 60 to bond the pre-sintered preform 11 to the tip.

In particular, as shown in Figure 5, the pre-sintered preform made of two layers is manufactured by a sequence of subsequent sintering processes. Each layer can be manufactured individually in a form of flexible sheet driven by a conveyor belt: namely by a bonding layer manufacturing process 201 and relative pre-sintering 203 and an abrasive layer manufacturing process 202 and relative pre-sintering 204. According to the bonding layer manufacturing process 201, the two metallic powders used to form the bonding layer 12 are mixed 2011 together with a binder to produce a paste which is pressed 2012 between opposite rollers. When the flexible sheet reaches the proper thickness, it is cut 2013 and weighted 2014 to form a tape. The sheet or tape is then pre-sintered 203, i.e. put in high vacuum furnace and vacuum heat treated 1150 - 1180 °C to obtain a pre-sintered sheet or tape. According to the abrasive layer manufacturing process 202, the cubic boron nitride (cBN) powder, the aluminum oxide (Al₂O₃) powder and the two metallic powders of same composition of the bonding layer used to form the abrasive layer 13 are mixed 2021 together with a binder to produce a paste which is pressed 2022 between opposite rollers. When the flexible sheet reaches the proper thickness, it is cut 2023 and weighted 2024 to form a tape. The sheet or tape is then pre-sintered 204, i.e. put in a high vacuum furnace and vacuum heat treated at 1150 - 1180 °C to obtain a pre-sintered sheet or tape. The two pre-sintered sheets or tapes are then placed 205 one on the top of the other to form a sheet or tape composed of a bonding layer 12 and a top layer 13 or abrasive layer 13. The sheet or tape is then sintered 30 to couple the two layers together in a high vacuum furnace, at pressure minor than 5 x 10E-4 torr and subsequently cut 40 to form the final pre-sintered preform 11.

Alternatively, according to an exemplary embodiment, as shown in Figures 6, the pre-sintered preform made of two layers is manufactured by simultaneously sintering the two layers. The two metallic powders used to form 206 the bonding layer 12 are mixed 2061 together with a binder to produce paste which is pressed 2062 between opposite rollers. When the flexible sheet reaches the proper thickness, the same mixing 2071 and pressing 2072 steps are performed to form 207 the abrasive layer 13 with embedded ceramic particles arranged on the top of the bonding layer 12. The two sheets are then simultaneously sintered 30 and coupled together in a high vacuum furnace, at pressure minor than 5 x 10E-4 torr and subsequently cut 40 to form the final pre-sintered preform 11.

According to an exemplary embodiment, the brazing step 60 of blade 10 with previously tack welded 50 preform 11 is carried out at 1200 - 1220 °C at a pressure lower than 5 x 10E-4 torr. According to an exemplary embodiment, also shown in Figure 6, subsequent sub-steps of reiterated heating 601 and diffusion 602 are carried out, at a temperature of the diffusion sub-step 602 between 1178 °C and 1198 °C, to realize proper bonding between preform 11 and blade 10. The brazing step is then concluded by quenching 603, lowering the temperature down to room temperature.

According to an exemplary embodiment, the brazing step 60 of blade 10 has to follow the following thermal cycle:
- heating up to 1038 °C in 150 minutes
- holding at 1038 °C for 30 minutes
- heating up to 1177 °C in 20 minutes
- holding at 1177 °C for 30 minutes
- heating up to 1218 °C in 5 minutes
- holding at 1218 °C for 20 ±5 minutes
- argon quenching to room temperature (1.2 ÷ 1.8 bar).
The aim of the heat treatment of the brazing step 60 is multiple:
- to bond ceramic particles with metallic matrix to reach abrasive properties needed by the blade to prevent excessive wear during run against statoric shroud;
- to minimize degradation of Nickel base superalloy, for instance the recrystallization of machined root.
The single furnace run of the assembly is aimed to get a lean process with reduced time compared to thermal sprayed or electrolytic abrasive coatings.

An important advantage of the exemplary embodiment of the pre-sintered preforms is the possibility of using such preforms at high temperature, tested up to 980 °C metal temperature. The pre-sintered preforms can also be produced as net shape preforms, in order to reduce waste and be flexible for the application on axial, radial and mixed turbomachines.

An additional application of the pre-sintered preforms according to the exemplary embodiments herein disclosed might be an assembly of combustion liner and transition piece which slide past each other, the transition piece channelling the high-temperature gas from the combustion liner to a first statoric nozzle of a gas turbine.

Another application of the pre-sintered preforms according to the exemplary embodiments herein disclosed on gas turbine blades might be angel wing seals between a rotor blade and nozzle in a turbine, which inhibits ingestion of hot gas from a hot gas flow through the turbine into turbine wheel spaces.

Still another application of the pre-sintered preforms according to the exemplary embodiments herein disclosed is to realize sealing among rotating turbine components, stationary nozzles, and casing of a gas turbine, such as on J-seals. It is known that J-seals are an integral part of efficient steam turbine operation. The failure of a J-seal can cause significant damage to a turbine rotor as material migrates downstream. For that reason, plant staff must conduct inspections of steam path systems to identify potential problems during regularly scheduled outages in order to check the integrity of the sealing. Steam turbine efficiency relies heavily on integrity and performance of steam path stage-to-stage seals. Using abrasive pre-sintered preforms according to the exemplary embodiments herein disclosed can result in a significant advantage in sealing among rotating turbine components, stationary nozzles, and casing by allowing for a long-lasting integrity of seals.

## Claims

1. An abrasive gas turbine blade tip cap preform (11) configured to bond to a gas turbine blade tip to form an abrasive gas turbine blade tip cap, the abrasive gas turbine blade tip cap preform (11) being formed of a bonding layer (12) and an abrasive layer (13), by the bonding layer (12) being a metallic layer comprising powder size particles of a nickel braze alloy and a nickel base superalloy, **characterized by**
the abrasive layer (13) being a ceramic layer in a metal matrix comprising powder size particles of cubic boron nitride (cBN) and aluminum oxide (Al₂O₃) in a metal matrix of same composition of the bonding layer (12);
wherein the abrasive layer (13) is composed of 25%±7.5% by weight of powder size particles of cubic boron nitride (cBN) and 25%±7.5% by weight of powder size particles of aluminum oxide (Al₂O₃) in 50%±15% by weight of a metal matrix, the metal matrix being composed of 50%±15% by weight of Ni based superalloy and 50%±15% by weight of Ni based braze alloy.

2. The abrasive gas turbine blade tip cap preform (11) of claim 1, wherein the thickness of the bonding layer (12) is 50%±15% of total thickness of the abrasive gas turbine blade tip cap preform (11).

3. The abrasive gas turbine blade tip cap preform (11) of claim 1, wherein the bonding layer (12) is composed of 50%±15% by weight of powder size particles of Ni based superalloy and 50%±15% by weight of powder size particles of Ni based braze alloy.

4. The abrasive gas turbine blade tip cap preform (11) of claim 1, wherein cubic boron nitride (cBN) particle size is in a range of 181-277 mesh in 93%wt minimum, aluminum oxide particle size is 100 mesh in 40%wt minimum, Ni based superalloy particle size is 395 mesh in 95%wt minimum and Ni based braze alloy particle size is 395 mesh in 95%wt minimum.

5. The abrasive gas turbine blade tip cap preform (11) of claim 1, wherein said nickel braze alloy is composed of: cobalt 13.5-16.5% by weight, chromium 18.5-21.5% by weight, aluminum 4.2-5.8% by weight, silicon 7.5-8.4% by weight, nickel 46.71-55.21% by weight, other elements less than 1.1% by weight.

6. The abrasive gas turbine blade tip cap preform (11) of claim 1, wherein said nickel based superalloy is composed of: cobalt 11.35-12.1% by weight, chromium 6.5-7.2% by weight, aluminum 5.9-6.6% by weight, tantalum 6.1-6.7% by weight, tungsten 4.5-5.3% by weight, hafnium 1.2-1.8% by weight, rhenium 2.5-3.1% by weight, nickel 55.61-60.36% by weight, other elements less than 1.6% by weight.

7. A method of manufacturing the abrasive gas turbine blade tip cap preform (11) of any one of claims 1-6, comprising the steps of:
- forming (20) a sheet or a tape formed of a bonding layer (12) and an abrasive layer (13), the bonding layer (12) comprising powder size particles of a nickel braze alloy and a nickel base superalloy, and the abrasive layer (13) comprising powder size particles of cubic boron nitride (cBN) and aluminum oxide (Al₂O₃) in a matrix of same composition of the bonding layer (12), said nickel braze alloy having a brazing temperature;
- vacuum heat treating (30) said sheet or tape at 80-90% of the brazing temperature; and
- cutting (40) said sheet or tape to the final shape of said abrasive gas turbine blade tip cap preform (11).

8. The method of manufacturing of claim 7, wherein the step of forming (20) the two layered sheet or tape alternatively comprises the steps of:
- forming (201) a bonding layer (12) comprising powder size particles of a nickel braze alloy and a nickel base superalloy;
- sintering (203) the bonding layer (12) by vacuum heat treating the bonding layer (12) at 80-90% of the brazing temperature;
- forming (202) an abrasive layer (13), the abrasive layer (13) comprising powder size particles of cubic boron nitride (cBN) and aluminum oxide (Al₂O₃) in a metal matrix of same composition of the bonding layer (12);
- sintering (204) the abrasive layer (13) by vacuum heat treating the abrasive layer (13) at 80-90% of the brazing temperature; and
- placing (205) the abrasive layer (13) on the top of the bonding layer (12);
or
- forming (206) a bonding layer (12) comprising powder size particles of a nickel braze alloy and a nickel base superalloy;
- forming (207) an abrasive layer (13), above the first layer, the abrasive layer (13) comprising powder size particles of cubic boron nitride (cBN) and aluminum oxide (Al₂O₃) in a matrix of same composition of ther bonding layer (12);
and additionally comprising the following steps:
- vacuum heat treating (30) said layers at 80-90% of the brazing temperature to form a metallic sheet; and
- cutting (40) the metallic sheet to desired shape.

9. A method of bonding the abrasive gas turbine blade tip cap preform (11) of claim 1 to a blade tip to form an abrasive blade tip cap comprising the step of:
- tack welding (50) said abrasive gas turbine blade tip cap preform (11) to the tip of a gas turbine blade (10);
- vacuum heat treating (60) to bond together the abrasive gas turbine blade tip cap preform (11) and the gas turbine blade tip by vacuum brazing.

10. The method of claim 9, wherein the step of vacuum heat treating (60) comprises reiterated sub-steps of heating (601) and diffusion (602), followed by a final sub-step of quenching (603) by lowering the temperature down to room temperature.

## Patentansprüche

1. Abrasive Gasturbinenschaufelspitzenkappenvorform (11), die konfiguriert ist, um an eine Gasturbinenschaufelspitze gebunden zu werden, um eine abrasive Gasturbinenschaufelspitzenkappe zu bilden, wobei die abrasive Gasturbinenschaufelspitzenkappenvorform (11) aus einer Bindungsschicht (12) und einer abrasiven Schicht (13) gebildet ist, wobei die Bindungsschicht (12) eine metallische Schicht ist, die Teilchen in Pulvergröße aus einer Nickelhartlötlegierung und einer nickelbasierten Superlegierung umfasst, **dadurch gekennzeichnet, dass** die abrasive Schicht (13) eine keramische Schicht in einer Metallmatrix ist, die Teilchen in Pulvergröße aus kubischem Bornitrid (cBN) und Aluminiumoxid (Al₂O₃) in einer Metallmatrix mit der gleichen Zusammensetzung wie die Bindungsschicht (12) umfasst;
wobei die abrasive Schicht (13) zu 25 Gew.-% ± 7,5 Gew.-% aus Teilchen in Pulvergröße aus kubischem Bornitrid (cBN) und zu 25 Gew.-% ± 7,5 Gew.-% aus Teilchen in Pulvergröße aus Aluminiumoxid (Al₂O₃) in 50 Gew.-% ± 15 Gew.-% einer Metallmatrix zusammengesetzt ist, wobei die Metallmatrix zu 50 Gew.-% ± 15 Gew.-% aus einer Ni-basierten Superlegierung und zu 50 Gew.-% ± 15 Gew.-% aus einer Ni-basierten Hartlötlegierung zusammengesetzt ist.

2. Abrasive Gasturbinenschaufelspitzenkappenvorform (11) nach Anspruch 1, wobei die Dicke der Bindungsschicht (12) 50 % ± 15 % der Gesamtdicke der abrasiven Gasturbinenschaufelspitzenkappenvorform (11) beträgt.

3. Abrasive Gasturbinenschaufelspitzenkappenvorform (11) nach Anspruch 1, wobei die Bindungsschicht (12) zu 50 Gew.% ± 15 Gew.-% aus Teilchen in Pulvergröße einer Ni-basierten Superlegierung und zu 50 Gew.-% ± 15 Gew.-% aus Teilchen in Pulvergröße einer Ni-basierten Hartlötlegierung zusammengesetzt ist.

4. Abrasive Gasturbinenschaufelspitzenkappenvorform (11) nach Anspruch 1, wobei die Größe der Teilchen aus kubischem Bornitrid (cBN) in einem Bereich von 181 bis 277 Mesh bei mindestens 93 Gew.-% beträgt, die Größe der Teilchen aus Aluminiumoxid 100 Mesh bei mindestens 40 Gew.-% beträgt, die Größe der Teilchen aus Ni-basierter Superlegierung 395 Mesh bei mindestens 95 Gew.-% beträgt und die Größe der Teilchen aus Ni-basierter Hartlötlegierung 395 Mesh bei mindestens 95 Gew.-% beträgt.

5. Abrasive Gasturbinenschaufelspitzenkappenvorform (11) nach Anspruch 1, wobei die Nickelhartlötlegierung zusammengesetzt ist aus: zu 13,5 bis 16,5 Gew.-% Kobalt, zu 18,5 bis 21,5 Gew.-% Chrom, zu 4,2 bis 5,8 Gew.-% Aluminium, zu 7,5 bis 8,4 Gew.-% Silizium, zu 46,71 bis 55,21 Gew.-% Nickel, zu weniger als 1,1 Gew.-% anderen Elementen.

6. Abrasive Gasturbinenschaufelspitzenkappenvorform (11) nach Anspruch 1, wobei die Ni-basierte Superlegierung zusammengesetzt ist aus: zu 11,35 bis 12,1 Gew.-% Kobalt, zu 6,5 bis 7,2 Gew.-% Chrom, zu 5,9 bis 6,6 Gew.-% Aluminium, zu 6,1 bis 6,7 Gew.-% Tantal, zu 4,5 bis 5,3 Gew.-% Wolfram, zu 1,2 bis 1,8 Gew.-% Hafnium, zu 2,5 bis 3,1 Gew.-% Rhenium, zu 55,61 bis 60,36 Gew.-% Nickel, zu weniger als 1,6 Gew.-% anderen Elementen.

7. Verfahren zur Herstellung einer abrasiven Gasturbinenschaufelspitzenkappenvorform (11) nach einem der Ansprüche 1 bis 6, umfassend die Schritte:
- Ausbilden (20) eines Blechs oder eines Bandes, das aus einer Bindungsschicht (12) und einer abrasiven Schicht (13) gebildet ist, wobei die Bindungsschicht (12) Teilchen in Pulvergröße einer Nickelhartlötlegierung und einer nickelbasierten Superlegierung umfasst und die abrasive Schicht (13) Teilchen in Pulvergröße aus kubischem Bornitrid (cBN) und Aluminiumoxid (Al₂O₃) in einer Matrix mit der gleichen Zusammensetzung wie die Bindungsschicht (12) umfasst, wobei die Nickelhartlötlegierung eine Löttemperatur aufweist;
- Vakuumwärmebehandeln (30) des Blechs oder Bandes bei 80 bis 90 % der Löttemperatur; und
- Schneiden (40) des Blechs oder Bandes in die endgültige Form der abrasiven Gasturbinenschaufelspitzenkappenvorform (11).

8. Verfahren nach Anspruch 7, wobei der Schritt des Ausbildens (20) des zweilagigen Blechs oder Bandes alternativ die Schritte umfasst:
- Ausbilden (201) einer Bindungsschicht (12), umfassend Teilchen in Pulvergröße einer Nickelhartlötlegierung und einer nickelbasierten Superlegierung;
- Sintern (203) der Bindungsschicht (12) durch Vakuumwärmebehandeln der Bindungsschicht (12) bei 80 bis 90 % der Löttemperatur;
- Ausbilden (202) einer abrasiven Schicht (13), wobei die abrasive Schicht (13) Teilchen in Pulvergröße aus kubischem Bornitrid (cBN) und Aluminiumoxid (Al₂O₃) in einer Metallmatrix mit der gleichen Zusammensetzung wie die Bindungsschicht (12) umfasst;
- Sintern (204) der abrasiven Schicht (13) durch Vakuumwärmebehandeln der abrasiven Schicht (13) bei 80 bis 90 % der Löttemperatur; und
- Anordnen (205) der abrasiven Schicht (13) auf der Oberseite der Bindungsschicht (12);
oder
- Ausbilden (206) einer Bindungsschicht (12), umfassend Teilchen in Pulvergröße einer Nickelhartlötlegierung und einer nickelbasierten Superlegierung;
- Ausbilden (207) einer abrasiven Schicht (13) über der ersten Schicht, wobei die abrasive Schicht (13) Teilchen in Pulvergröße aus kubischem Bornitrid (cBN) und Aluminiumoxid (Al₂O₃) in einer Matrix mit der gleichen Zusammensetzung wie die Bindungsschicht (12) umfasst;
und zusätzlich die folgenden Schritte umfassend:
- Vakuumwärmebehandeln (30) der Schichten bei 80 bis 90 % der Löttemperatur, um ein Metallblech zu bilden; und
- Schneiden (40) des Metallblechs in die gewünschte Form.

9. Verfahren zum Binden der abrasiven Gasturbinenschaufelspitzenkappenvorform (11) nach Anspruch 1 an eine Schaufelspitze, um eine abrasive Schaufelspitzenkappe zu bilden, umfassend den Schritt:
- Heftschweißen (50) der abrasiven Gasturbinenschaufelspitzenkappenvorform (11) an die Spitze einer Gasturbinenschaufel (10);
- Vakuumwärmebehandeln (60), um die abrasive Gasturbinenschaufelspitzenkappenvorform (11) und die Gasturbinenschaufelspitze durch Vakuumlöten aneinander zu binden.

10. Verfahren nach Anspruch 9, wobei der Schritt des Vakuumwärmebehandelns (60) wiederholte Unterschritte des Erwärmens (601) und der Diffusion (602) umfasst, gefolgt von einem abschließenden Unterschritt des Abschreckens (603) durch Absenken der Temperatur auf Raumtemperatur.

## Revendications

1. Préforme (11) de capuchon abrasif d'extrémité d'aube de turbine à gaz configurée pour se lier à une extrémité d'aube de turbine à gaz pour former un capuchon abrasif d'extrémité d'aube de turbine à gaz, la préforme (11) de capuchon abrasif d'extrémité d'aube de turbine à gaz étant formée d'une couche de liaison (12) et d'une couche abrasive (13), la couche de liaison (12) étant une couche métallique comprenant des particules pulvérulentes d'un alliage de brasage à base de nickel et d'un superalliage à base de nickel,
**caractérisée en ce que** la couche abrasive (13) est une couche céramique dans une matrice métallique comprenant des particules pulvérulentes de nitrure de bore cubique (cBN) et d'oxyde d'aluminium (Al₂O₃) dans une matrice métallique de même composition que celle de la couche de liaison (12) ;
dans laquelle la couche abrasive (13) est composée de 25 %±7,5 % en poids de particules pulvérulentes de nitrure de bore cubique (cBN) et de 25 %±7,5 % en poids de particules pulvérulentes d'oxyde d'aluminium (Al₂O₃) dans 50 %±15 % en poids d'une matrice métallique, la matrice métallique étant composée de 50 %±15 % en poids de superalliage à base de Ni et de 50 %±15 % en poids d'alliage de brasage à base de Ni.

2. Préforme (11) de capuchon abrasif d'extrémité d'aube de turbine à gaz selon la revendication 1, dans laquelle l'épaisseur de la couche de liaison (12) est de 50 %±15 % de l'épaisseur totale de la préforme (11) de capuchon abrasif d'extrémité d'aube de turbine à gaz.

3. Préforme (11) de capuchon abrasif d'extrémité d'aube de turbine à gaz selon la revendication 1, dans laquelle la couche de liaison (12) est composée de 50 %±15 % en poids de particules pulvérentes de superalliage à base de Ni et de 50 %±15 % en poids de particules pulvérentes d'alliage de brasage à base de Ni.

4. Préforme (11) de capuchon abrasif d'extrémité d'aube de turbine à gaz selon la revendication 1, dans laquelle la taille des particules de nitrure de bore cubique (cBN) se situe dans une plage allant de 181 à 277 mesh à 93 % en poids minimum, la taille des particules d'oxyde d'aluminium est de 100 mesh à 40 % en poids minimum, la taille des particules de superalliage à base de Ni est de 395 mesh à 95 % en poids minimum et la taille des particules d'alliage de brasage à base de Ni est de 395 mesh à 95 % en poids minimum.

5. Préforme (11) de capuchon abrasif d'extrémité d'aube de turbine à gaz selon la revendication 1, dans laquelle ledit alliage de brasage à base de nickel est composé de : cobalt à 13,5-16,5 % en poids, chrome à 18,5-21,5 % en poids, aluminium à 4,2-5,8 % en poids, silicium à 7,5-8,4 % en poids, nickel à 46,71-55,21 % en poids, autres éléments à moins de 1,1 % en poids.

6. Préforme (11) de capuchon abrasif d'extrémité d'aube de turbine à gaz selon la revendication 1, dans laquelle ledit superalliage à base de nickel est composé de : cobalt à 11,35-12,1 % en poids, chrome à 6,5-7,2 % en poids, aluminium à 5,9-6,6 % en poids, tantale à 6,1-6,7 % en poids, tungstène à 4,5-5,3 % en poids, hafnium à 1,2-1,8 % en poids, rhénium à 2,5-3,1 % en poids, nickel à 55,61-60,36 % en poids, autres éléments à moins de 1,6 % en poids.

7. Procédé pour la fabrication de la préforme (11) de capuchon abrasif d'extrémité d'aube de turbine à gaz selon l'une quelconque des revendications 1 à 6, comprenant les étapes consistant à :
- former (20) une feuille ou une bande formée d'une couche de liaison (12) et d'une couche abrasive (13), la couche de liaison (12) comprenant des particules pulvérentes d'un alliage de brasage à base de nickel et d'un superalliage à base de nickel, et la couche abrasive (13) comprenant des particules pulvérentes de nitrure de bore cubique (cBN) et d'oxyde d'aluminium (Al₂O₃) dans une matrice de même composition que celle de la couche de liaison (12), ledit alliage de brasage à base de nickel présentant une température de brasage ;
- traitement thermique sous vide (30) de ladite feuille ou bande à 80-90 % de la température de brasage ; et
- couper (40) ladite feuille ou bande à la forme finale de ladite préforme (11) de capuchon abrasif d'extrémité d'aube de turbine à gaz.

8. Procédé pour la fabrication selon la revendication 7, dans lequel l'étape de formation (20) de la feuille ou de la bande à deux couches comprend alternativement les étapes consistant à :
- former (201) une couche de liaison (12) comprenant des particules pulvérentes d'un alliage de brasage à base de nickel et d'un superalliage à base de nickel ;
- fritter (203) la couche de liaison (12) par traitement thermique sous vide de la couche de liaison (12) à 80-90 % de la température de brasage ;
- former (202) une couche abrasive (13), la couche abrasive (13) comprenant des particules pulvérentes de nitrure de bore cubique (cBN) et d'oxyde d'aluminium (Al₂O₃) dans une matrice métallique de même composition que celle de la couche de liaison (12) ;
- fritter (204) la couche abrasive (13) par traitement thermique sous vide de la couche abrasive (13) à 80-90 % de la température de brasage ; et
- placer (205) la couche abrasive (13) sur la couche de liaison (12) ;
ou
- former (206) une couche de liaison (12) comprenant des particules pulvérentes d'un alliage de brasage à base de nickel et d'un superalliage à base de nickel ;
- former (207) une couche abrasive (13), au-dessus de la première couche, la couche abrasive (13) comprenant des particules pulvérentes de nitrure de bore cubique (cBN) et d'oxyde d'aluminium (Al₂O₃) dans une matrice de même composition que celle de la couche de liaison (12) ;
et comprenant en outre les étapes suivantes :
- traitement thermique sous vide (30) desdites couches à 80-90 % de la température de brasage pour former une feuille métallique ; et
- découpe (40) de la feuille métallique à la forme souhaitée.

9. Procédé pour la liaison de la préforme (11) de capuchon abrasif d'extrémité d'aube de turbine à gaz selon la revendication 1 sur une extrémité d'aube pour former un capuchon abrasif d'extrémité d'aube, comprenant l'étape consistant à :
- souder par pointage (50) ladite préforme (11) de capuchon abrasif d'extrémité d'aube de turbine à gaz à l'extrémité d'une aube de turbine à gaz (10) ;
- la traiter de façon thermique sous vide (60) pour lier ensemble la préforme (11) de capuchon abrasif d'extrémité d'aube de turbine à gaz et l'aube de turbine à gaz par brasage sous vide.

10. Procédé selon la revendication 9, dans lequel l'étape de traitement thermique sous vide (60) comprend des sous-étapes répétées de chauffage (601) et de diffusion (602), suivies d'une sous-étape finale de trempe (603) par abaissement de la température jusqu'à la température ambiante.
